

May 8, 1951

E. E. HOWARD ET AL  
ABRASIVE TOOL COMPRISING BONDED ABRASIVE ELEMENTS  
CEMENTED TO SUPPORTING ELEMENTS  
Filed Jan. 23, 1947

2,552,485



Inventors  
ELMER E. HOWARD  
GEORGE J. GOEPFERT  
by *W. J. Wiley*  
Attorney

## UNITED STATES PATENT OFFICE

2,552,485

ABRASIVE TOOL COMPRISING BONDED  
ABRASIVE ELEMENT CEMENTED TO  
SUPPORTING ELEMENT

Elmer E. Howard, Buffalo, and George J. Goepfert, Niagara Falls, N. Y., assignors to The Carborundum Company, Niagara Falls, N. Y., a corporation of Delaware

Application January 23, 1947, Serial No. 723,774

6 Claims. (Cl. 51—298)

1

This invention relates to abrasive tools comprising a bonded abrasive element attached to a rigid supporting element by a cement comprising a phenol-aldehyde condensation product and a partial acetal of polyvinyl alcohol. It is especially concerned with such tools wherein the abrasive of the bonded abrasive element comprises a substantial proportion of diamonds.

Because of the relatively high cost of diamonds, where they are employed for abrasive purposes they are usually sold in the form of a tool comprising a supporting element and an abrasive element which is formed by bonding either the diamonds alone or mixtures of diamonds with other conventional abrasive materials. The bond of the abrasive element may be metal, a resin such as heat-hardened phenolic condensation product, or a vitrified material. The backing elements are usually either a metal such as steel or an aluminum alloy or a molded phenol resin containing a reinforcing filler such as comminuted fabric or powdered metal. The various types of abrasive elements may be attached to the different backings, as for example, metal, vitrified, or resin bonded abrasive elements may be used with either the metallic or the molded resin backings. For that reason and because of the stresses set up in the cement during both the manufacture and the use of the abrasive tool, the development of a satisfactory cement has presented a serious and difficult problem. Our invention provides a solution for that problem.

It is accordingly an object of the present invention to provide an abrasive tool in which a bonded abrasive element is attached to a supporting backing by a cement which will have the necessary strength and heat resistance to withstand the stresses set up in such a cement during the production and use of such abrasive tool. Another object of the invention is to provide an abrasive tool in which a bonded abrasive element is cemented to a supporting element by a cement comprising a phenolic resin and a partial acetal of polyvinyl alcohol. Other objects of the invention will appear from the disclosure following hereinafter.

We have discovered that abrading tools of many different shapes and for many different purposes can be satisfactorily made by cementing abrasive elements to supporting elements by a cement comprising the heat-hardened reaction product of a liquid comprising a phenol-aldehyde condensation product and a partial acetal of polyvinyl alcohol. Although we may employ various phenolic resins and different acetals of polyvinyl

2

alcohol, we have found that a cement prepared by admixing a solution of a butyraldehyde partial acetal of polyvinyl alcohol with a phenol-aldehyde resin in the A stage is especially satisfactory for use in our invention.

Understanding of the invention will be facilitated by reference to the accompanying drawings, wherein:

Figure 1 is a top plan view of a cup wheel made in accordance with one embodiment of the invention;

Figure 2 is a section on the lines 2—2 of Figure 1;

Figure 3 is a side elevation of a tool for grinding tapered holes in glassware;

Figure 4 is a bottom plan view of the tool of Figure 3;

Figure 5 is a side elevation of an abrasive element employed in the tool of Figures 3 and 4;

Figure 6 is an end elevation of the abrasive element of Figure 5;

Figure 7 is a plan view of a ring in which abrasive elements may be mounted to form a segmental grinding tool;

Figure 8 is a side elevation of the ring of Figure 7 showing the abrasive elements mounted therein; and

Figure 9 is a section of a tool designed forlapping glass lenses.

Referring to the drawings, the cup wheel of Figures 1 and 2 comprises a supporting element 1 made by molding a mixture of phenolic resin and powdered aluminum filler and being provided with an arbor hole 2 for mounting. An abrasive ring 3 is cemented to the top of the cup by cement 4.

The tool of Figures 3 and 4 comprises a truncated cone 6 provided with a driving spindle 7 and having abrasive elements 8 mounted in recesses in the exterior surface of the cone by cement 4.

Figures 5 and 6 are side and end elevations, respectively, of abrasive elements adapted for use in the tool of Figures 3 and 4. The elements comprise a metal portion 9 and a metal bonded abrasive portion 10. The two portions are formed as an integral element by placing powdered metal in a mold in an amount to form the portion 9, putting thereover a quantity of powdered metal containing diamonds to form the abrasive portion 10, and pressing and sintering the mold contents to flux the powdered metal particles together.

The ring of Figure 7 comprises a steel ring 11 having bolt holes 12 extending part way up from

the bottom and recesses 13 separated by lands 14. The recesses are designed for receiving bonded abrasive elements. Figure 8 shows a side elevation of the ring of Figure 7 in which abrasive elements 15 have been cemented by cement 4.

The abrasive tool of Figure 9 comprises a supporting element 17 formed by molding and heat-hardening a mixture of phenolic resin provided with a comminuted fabric filler and provided with an arbor hole 18. An abrasive ring 19 is cemented to the upper surface of the supporting element by the cement 4.

Various features and embodiments of our invention are described in the following examples, which it is to be understood are for illustrative purposes only and are not limitative.

#### Example I

A cement was prepared by first reacting 343 parts of phenol, 236 parts of a 40% solution of formaldehyde in water and 3.4 parts of sodium hydroxide. The above mixture was heated for approximately 4 hours. At the end of this period substantially all of the formaldehyde had reacted with the phenol. The liquid resin so obtained was vacuum distilled at a pressure of 40-50 mm. until a resin temperature of 90° C. was reached. At the end of this period, the resin was further heated at atmospheric pressure for approximately 45 minutes at 130° C. Alcohol was added to thin the resin to yield a resin solution having a 32% solid content. To 100 parts of the resin solution so prepared were added 260 parts of a 12% alcohol solution of polyvinyl butyral resin designated as "XYNC" by the Carbide and Carbon Chemicals Corporation and 5 parts of paraformaldehyde. This polyvinyl butyral resin contained approximately 35 parts of butyraldehyde per 100 parts of original resin.

#### Example II

A cement was prepared by first reacting 285 parts of phenol, 165 parts of a 40% solution of formaldehyde in water and 8.6 parts of oxalic acid-dihydrate. The above mixture was heated under reflux for approximately 4 hours. At the end of this period substantially all of the formaldehyde had reacted with the phenol. The liquid resin so obtained was vacuum distilled and heat treated in the same way as the alkaline catalyzed liquid resin described in Example I above. At the end of this period alcohol was added to the resin to yield a resin solution having a 45% solid content. To 100 parts of the resin solution so prepared were added 38 parts of a 12% alcohol solution of polyvinyl butyral resin designated as "XYNC" by the Carbide and Carbon Chemicals Corporation and 7 parts of paraformaldehyde.

#### Example III

A cresylic acid-phenol formaldehyde resin was prepared by reacting 280 parts of phenol, 120 parts of p cresol, 421 parts of a 40% solution of formaldehyde in water and 8 parts of sodium hydroxide. The above mixture was heated at 55-60° C. for 24 hours. At the end of this period approximately 1-2% of the original amount of formaldehyde added had not reacted. The sodium hydroxide catalyst was then neutralized with dilute acetic acid. The neutral resin was vacuum distilled at a pressure of 30-40 mm. until a resin temperature of approximately 80° C. was reached. 20 parts of p cresol for each 100 parts of resin was added and the mixture was then

heated under atmospheric pressure for approximately 1/2 hour at 140° C. To 100 parts of the resin so obtained were added 2500 parts of a 12% solution of polyvinyl butyral resin of Example I in alcohol. The resulting mixture was used as a cement.

#### Example IV

An abrasive tool of the type illustrated in Figures 1 and 2, in which a metal bonded diamond abrasive element was cemented to a backing of a cast aluminum alloy, was prepared as follows:

A backing element 6 inches in diameter and having a width of 1/2 inch for the surface to which the abrasive ring was to be cemented was cast from an alloy sold commercially by the Frontier Bronze Corporation under the designation "Frontier 40 E." The alloy conforms to the ASTM specification for "Alloy O, B26-42T" and had the following chemical analysis:

|          |           |
|----------|-----------|
| Zn, 5.50 | Cu, 0.40  |
| Mg, 0.50 | Si, 0.30  |
| Cr, 0.50 | Mn, 0.30  |
| Ti, 0.20 | Al, 91.30 |
| Fe, 1.00 |           |

A ring having an outside diameter of 6 inches and an inside diameter of 5 inches to correspond to the mounting surface of the abrasive element was prepared as follows:

A mixture of metal powders comprising 90% copper and 10% tin was placed in a mold and suitably leveled. This mixture was then partially compacted and the abrasive mix was then placed on top. The abrasive mix comprised diamond particles of 100 grit size and powdered copper and tin powders of similar composition as the non-abrasive portion. The weight of metal powder was roughly 7 times the weight of the diamond abrasive portion. After suitable leveling, the metal powder mixture was compacted in the mold at 15 tons pressure per square inch of mold area.

The compacted ring was removed from the mold and sintered at 700° C. for sufficient time to flux the metal powder components and yield a suitable bond for the diamond abrasive. The non-abrasive portion of the ring was roughened on its face prior to cementing. The cement employed was prepared by thinning 37 parts by weight of a liquid composition prepared similarly to that described in Example I but sold commercially by the Bakelite Corporation under the designation "XJ17601" with 32 parts each of acetone and benzol. The resulting cement had a viscosity of 422 cp. at 25° C. This resin has a ratio of phenol-formaldehyde resin to polyvinyl butyral acetal approximately the same as that of Example III.

Both the abrasive element and the corresponding part of the supporting element were given two thin coats of the cement, allowing 15 minutes for each coat to dry by standing in the air. The abrasive ring was then placed on the supporting element with the adhesive coated surfaces together and the assemblage was hot pressed at a pressure of 300 pounds per square inch, calculated on the area of the cemented surfaces, between steam heated platens provided with steam under a pressure of 90 pounds (corresponding to 320° F.) for 30 minutes. The steam was then turned off and cooling water was run into the platens. The assemblage was left in the press until it had cooled to the point where it could be handled by hand without gloves whereupon

the pressure was relieved and the article was removed from the mold.

Tests of specially designed test pieces made from the same materials and according to the practice of this example showed a tensile strength at room temperature in excess of 1500 pounds per square inch and 550 pounds per square inch at a temperature of 300° F. The abrasive element was very strongly attached to the supporting element and the tool was very satisfactory for the purpose intended. 10

*Example V*

An abrasive tool for grinding the stopper holes in the necks of glass bottles was made of the form illustrated in Figures 3 and 4 with abrasive elements of the type illustrated in Figures 5 and 6.

As illustrated in Figures 3 and 4, the supporting element, which was made of steel, comprised a truncated cone having a length of 1 inch, a diameter at the top of 1 inch, and at the bottom of  $\frac{3}{4}$  inch. Three equally spaced recesses  $\frac{1}{8}$  inch wide and  $\frac{1}{16}$  inch deep were provided along the length of the periphery of the cone which had a driving spindle at the upper or larger end for mounting the tool in a chuck.

The abrasive elements, which were 1 inch long and  $\frac{1}{8}$  inch square, were formed in a manner similar to that described in Example IV except that approximately one-half of the total thickness of  $\frac{1}{8}$  inch of the abrasive sticks shown in Figures 5 and 6 consisted of the metal powder without the diamonds (9 of Figures 5 and 6) while the abrasive part 10, which was also approximately  $\frac{1}{16}$  inch thick, was of a powdered metal-diamond mix of the composition described in Example IV.

The recesses in the supporting element 6 and the metallic portion 9 of the sticks were given two coats of the cement of Example II, drying about 15 minutes after the application of each coat. The abrasive elements were then set into the recesses in the supporting tool, the assemblage was placed in a mold having an inside diameter of 1 inch with the longitudinal axis of the supporting element parallel to that of the hole in the mold. A weight of 5 pounds was then put on the upper flat surface of the supporting element to press the abrasive elements against the supporting element and the assemblage was put into an oven having a temperature of 320° F. for 30 minutes to heat-harden the resin cement. The assembly was removed and allowed to cool and the completed tool removed. It was found that the abrasive elements were strongly attached to the supporting element and the tool was very satisfactory for the purpose intended.

*Example VI*

A segmental disc wheel adapted for surfacing glass was made according to the design illustrated in Figures 7 and 8. A steel ring of a type sold for use in "Blanchard" disc grinders and having an outside diameter of 11 inches and an inside diameter of 9 inches was employed as the supporting element. The upper surface of the ring was provided with recesses  $\frac{1}{8}$  inch wide and  $\frac{1}{16}$  inch deep which were separated by lands approximately  $\frac{3}{4}$  inch long on the inner surface. The recesses were tangential to circles concentric with the ring, the larger one of which was 6 inches in diameter. Metal bonded diamond hones 1 inch by  $\frac{1}{2}$  inch by  $\frac{1}{2}$  inch were pressed as described in Example IV and one surface of these hones and the recesses of the ring were 70

coated with cement as described in the previous examples.

The abrasive elements were assembled in the recesses in the ring and the assemblage was then hot pressed as described in Example IV. After coating the article was removed from the press and it was found that the abrasive elements were very securely attached to the ring.

*Example VII*

A lap for grinding lenses and having the form illustrated in Figure 9 was prepared as follows:

The supporting element 17 was molded from a resin-communited fabric composition which is 15 a molding compound which was designed to have high impact strength. The element had an outside diameter of 3 inches and an inside diameter of  $2\frac{1}{2}$  inches.

A resin bonded diamond abrasive element 19 20 was prepared from a mixture of the following composition:

50 parts by weight—100 mesh size diamond bort  
3 parts by weight—liquid phenol-formaldehyde resin (sold by The Bakelite Corporation under the designation "Bakelite No. XR7534")  
25 22 parts by weight—powdered phenol-formaldehyde resin (sold by The Bakelite Corporation under the designation "Bakelite No. BR2428")  
30 25 parts by weight—powdered cryolite filler

A ring  $\frac{1}{4}$  inch thick and of a diameter to match the supporting element was pressed from this mixture and the article was heated to cure the resin bond.

35 The mold surface of the abrasive element and the upper surface of the supporting element were suitably cleaned and coated with two coats of the cement used in the preceding examples, drying as there described. The abrasive ring was then 40 put on the supporting element and the assemblage was hot pressed at a temperature of 320° F. for 30 minutes. After cooling, it was found that the abrasive element was very strongly secured to the supporting element and the tool was wholly satisfactory.

*Example VIII*

A resin bonded abrasive disc which contained 50 35% of 180 grit diamond bort, 25% of a phenol-aldehyde resin bond and 40% secondary grain and filler was cemented to a steel backing with the cement prepared from the "Bakelite resin XJ-17601" as described above. A steel disc  $\frac{1}{2}$  inch thick and 1 inch in diameter and provided 55 with a threaded spindle having a diameter of  $\frac{1}{2}$  inch was sandblasted to roughen one of the flat surfaces and, after cleaning, that surface was coated with two coats of cement, air drying each coat for about 15 minutes as described.

60 One of the flat surfaces of the resin bonded disc was thoroughly cleaned and similarly coated with cement, the elements were assembled and hot pressed as described in Example IV. After the cement had been cured and the article cooled, 65 it was found that the abrasive element was very strongly attached to the steel backing and that the cement had sufficient toughness and resilience so that the disc withstood very severe abrading operations.

*Example IX*

A diamond hone was made as follows:

A vitrified bonded diamond stick  $1\frac{1}{2}$  inches long,  $\frac{1}{4}$  inch wide and  $\frac{1}{16}$  inch thick was made 75 as follows:

A bond mix was prepared by ball-milling together

|                     | Parts by weight |
|---------------------|-----------------|
| Blended spar        | 5.7             |
| Tennessee ball clay | 11.4            |
| California talc     | 77.9            |
| 320 Silicon Carbide | 5.0             |

71 parts by weight of this mix was then mixed with 29 parts by weight of 220 grit diamond bort and 5 parts of water to make a moldable mass. A stick was molded from the mix under a pressure of 2000 pounds per square inch, and the formed stick was removed from the mold and fired in a kiln to vitrify the bond.

The stick was wet-disked to flatten the surfaces and was then dried for 16 hours at 150° F. and air blasted to clean it off. One of the 1½ by ¼ inch surfaces was given two coats of the cement, each of which was air dried for 15 minutes, and the abrasive element was then put into a mold 6 inches long by ¼ inch wide with the cement surface up. A sufficient quantity of a mixture containing 20% of a finely pulverized phenol-formaldehyde resin in the "A" stage and 80% of granular aluminum of the type known as "atomized metal powder" and having a particle size such that all of the powder passed through a 100 mesh screen to form a stick ¼ inch thick was then put into the mold. The top of the mix was leveled off, a plunger was placed on the mix and the assemblage was hot pressed under a pressure of 25 pounds per square inch for 5 minutes and for an additional 30 minutes at 2000 pounds per square inch. The steam was then turned off, the platens of the press were filled with cooling water, and the mold with its contents was removed from the press after the mold had cooled to the point where it could be handled without gloves.

After removing the hone from the mold it was disked to finish it to dimensions and the non-abrasive portion forming the handle was sanded and lacquered. The resulting product was very satisfactory, the abrasive element being strongly attached to the handle.

The cements employed in making our improved abrasive tools are very strong and tough. They are sufficiently tacky in the liquid condition after the solvent has been partially evaporated, as by air drying for 15 minutes, so that the abrasive elements are held in place strongly enough to permit handling without having the abrasive elements drop off or become displaced with respect to the backing element. This is a decided advantage in making many types of tools such as the bottle neck grinding tool of Example V and the segmental disc of Example VI.

When they are cured, these cements are strongly adherent to various types of supporting elements and bonded abrasives which are commonly used in making many types of tools. They are also very strong and tough and possess sufficient resilience so that they will absorb the stresses occasioned by the difference in coefficient of expansion between the various types of elements and backings and are thus highly resistant to shock. This characteristic makes them very well suited for many operations where the grinding elements are subjected to shock and the accompanying stresses. This is in marked contrast to the ordinary phenol-formaldehyde resin which has very poor resilience and is poorly adhesive to many types of surfaces. The cements are also heat-resistant, presumably because of the fact

that the phenolic constituent sets up to an infusible condition. This property is particularly valuable where the tools are used without coolant and are likely to get quite hot.

Various modifications of our invention may be made. The phenol-formaldehyde resin modified by the partial butyraldehyde acetal of polyvinyl alcohol is very well suited for use in our invention but other acetals such as those formed by acetalizing polyvinyl alcohol with formaldehyde and with acetaldehyde may also be used. The acetal does not necessarily have the extent of acetalization described in the specific examples, although in general we prefer to use rather highly acetalized compounds derived from polyvinyl alcohol of comparatively high molecular weight because such compounds have relatively high softening points and do not materially reduce the heat resistance of the phenolic component.

While there may be some reaction between the acetal and the phenolic resin during the final curing, the liquid cement composition is apparently merely a homogeneous mixture of the phenol-aldehyde liquid resin and the acetal. Such mixture may be made by dissolving the acetal, which is a solid at ordinary temperatures, in a solvent which is compatible with the liquid resin and blending the constituents in this manner. Alternatively the acetal, preferably in powdered form, may be admixed with the phenol and formaldehyde and the resin-forming reaction brought about in such mixture as a result of which the acetal apparently dissolves in the liquid resin. We have obtained satisfactory results with compositions made by both these methods.

Although in general we have not found it necessary to use fillers, the cements may be modified by the addition of comminuted fillers such as pulverized cryolite or flint or organic fillers such as cotton flock or wood flour in making some forms of abrasive tools in accordance with our invention.

In the claims where we have referred to an acetal as being acetalized to a certain percentage we mean that the acetal is of such composition that upon hydrolysis it yields that amount of the aldehyde. For example, if 100 parts of acetal are hydrolyzed and 35 parts of aldehyde are recovered, we would describe that as an acetal which had been acetalized 35%.

While we have described our invention by a number of specific examples, it is to be understood that it is not limited thereto but may be otherwise modified, the scope of the invention being defined by the appended claims.

We claim:

1. An abrasive tool adapted for both wet and dry grinding comprising a bonded abrasive element attached to a rigid supporting element by a cement comprising the solidified and heat-hardened reaction product of a liquid comprising about 100 parts of a normally liquid phenol-formaldehyde condensation product, about 10-400 parts of a water-insoluble partial acetal of polyvinyl alcohol and an aldehyde selected from the group consisting of butyraldehyde, formaldehyde and acetaldehyde and a volatile solvent, said cement having the characteristic of air drying to a tacky condition such that the abrasive elements are held in place strongly enough to permit handling without displacement of the said elements with respect to the backing element and in a cured condition being strongly adherent to various types of supporting elements and bonded abrasives, strong enough and of sufficient resili-

ence to absorb the stresses occasioned by the difference in coefficient of the expansion between the abrasive element and the backing and in the use of the tool, highly resistant to shock, and having sufficient heat-resistance to permit use of the tool for dry grinding and sufficient moisture-resistance to withstand the coolants used in wet grinding.

2. An article as claimed in claim 1 wherein the aldehyde of the partial acetal is butyraldehyde.

3. An article as claimed in claim 2 wherein the ratio of the phenol-formaldehyde condensation product to the partial acetal is about 1 to 1-3.

4. An article as claimed in claim 3 wherein the acetal is approximately 35% acetalized and has a molecular weight such that a 7.5% solution of the acetal in alcohol has a viscosity of 250 centipoises at 25° C.

5. An article as claimed in claim 1 wherein the aldehyde of the partial acetal is formaldehyde.

6. An article as claimed in claim 1 wherein the aldehyde of the partial acetal is acetaldehyde.

ELMER E. HOWARD,  
GEORGE J. GOEPFERT.

## REFERENCES CITED

The following references are of record in the file of this patent:

## UNITED STATES PATENTS

| Number    | Name           | Date          |
|-----------|----------------|---------------|
| 1,832,515 | Webster        | Nov. 17, 1931 |
| 2,111,006 | Robie          | Mar. 15, 1938 |
| 2,261,983 | Ford           | Nov. 11, 1941 |
| 2,307,588 | Jackson et al. | Jan. 5, 1943  |
| 2,387,831 | Cogan et al.   | Oct. 30, 1945 |
| 2,416,182 | Kistler        | Feb. 18, 1947 |

## OTHER REFERENCES

20 Ser. No. 301,165, Puizer-Reybegg (A. P. C.), published Apr. 20, 1943.